

## UNITED STATES PATENT OFFICE.

JOHN M. SKILLING, OF WILMINGTON, DELAWARE, ASSIGNOR TO E. I. DU PONT DE NEMOURS & COMPANY, OF WILMINGTON, DELAWARE, A CORPORATION OF DELAWARE.

## PROGRESSIVE NITROCELLULOSE POWDER CONTAINING NITROGUANIDINE.

No Drawing.

Application filed June 15, 1922. Serial No. 568,597.

*To all whom it may concern:*

Be it known that I, JOHN M. SKILLING, a citizen of the United States, and a resident of Wilmington, in the county of New Castle 5 and State of Delaware, have invented certain new and useful Progressive Nitrocellulose Powders Containing Nitroguanidine, of which the following is a specification.

This invention relates to progressive nitrocellulose powders containing a substantial proportion of nitroguanidine, and to a process of making such powders.

The object of my invention is to surface-impregnate with deterrent materials the surface of smokeless powder grains made from a composition in which a substantial proportion of the nitrocellulose is replaced by nitroguanidine. The substitution of nitroguanidine for a portion of the nitrocellulose 15 gives a powder with lower temperature of combustion and consequently a powder which produces less erosion. This improvement alone constitutes a very substantial improvement over existing powders made of nitrocellulose alone or a mixture of nitrocellulose and nitroglycerine as a base. I have found that still further ballistic improvement is possible by impregnating the surface of the powder grains with deterrent 20 materials having at least some solvent action on the nitrocellulose portion of the powder grains whereby the initial combustion of the powder is retarded and the powder burns more progressively as is characteristic of nitrocellulose powders thus treated.

The powder which I surface impregnate with deterrent materials may be made according to the procedure prescribed in my copending application, U. S. Serial No. 40 535,315, filed February 9, 1922, such a powder containing from 30 to 80% nitrocellulose, and from 70 to 20% nitroguanidine. For example, I may make up a powder composed of 45 60 parts nitrocellulose, having a nitrogen content in the neighborhood of 13.0% and a solubility in a mixture of 2 parts ethyl ether to 1 part ethyl alcohol in the neighborhood of 40%, and 40 parts finely divided nitroguanidine and 0.5 parts of diphenylamine, as 50 a stabilizing agent, to 100 parts of composition and with or without the addition of nitrohydrocarbons and other ingredients added for various purposes, such as reducing the hygroscopic qualities of the composition. I

may colloid such a composition with a mixture of 55 2 parts ethyl ether to 1 part ethyl alcohol, and press through a die with an external diameter of .05" provided with central pin .015" in diameter. The strings of colloid from the above die, I may granulate 60 in any convenient length, such as 1/11". The granulated powder is then placed in solvent recovery for several days for the purpose of recovering ether and alcohol. The powder is then dried, preferably at a temperature below 65° C. until the residual alcohol and ether remaining in the powder is reduced to the amount desired, generally below 2.0%.

I then take the powder prepared in the 70 above manner and surface impregnate it with a deterrent material, such as dinitrotoluene (1-2-4). As the nitroguanidine component of the powder grain is appreciably soluble 75 in water and the solubility increases with the temperature of the water, I prefer to use a surface impregnating treatment which does not remove a substantial amount of nitroguanidine from the powder. For example, 80 100 parts of the powder grains to be surface impregnated may be placed in a rotating pan or bowl. From 3.5 to 5 parts of finely divided 1, 2, 4-dinitrotoluene are then added and the container rotated until the powder grains and dinitrotoluene are thoroughly 85 mixed. A jet of live steam is then directed into the rotating container, gradually raising the temperature of the mixture of dinitrotoluene and powder until the dinitrotoluene is melted and caused to impregnate 90 the surface of the powder grains because of its solvent action on the nitrocellulose. Care is taken during this treatment to prevent excessive condensation of steam, as I desire to prevent as far as possible the extraction of 95 the nitroguanidine component of the powder grain. A small amount of dinitrotoluene in excess of the amount to be incorporated is usually added to the mixing vessel to take care of mechanical losses; thus 4.1 parts may 100 be added when it is intended to have the resulting powder contain 4 parts of deterrent.

The effect of surface impregnating the powder grains with the dinitrotoluene is illustrated by the following ballistic results in 105 the .30/06 Springfield rifle using the 180-grain bullet. The powder before being surface-impregnated with dinitrotoluene gave,

with a weight of charge of 47.0 grains, an instrumental velocity at 78 feet of 2380 f. s. with a mean pressure of 48,140 pounds per square inch. After surface impregnating 5 the powder grains with approximately 4 parts dinitrotoluene to 100 parts of powder, the impregnated powder, with a weight of charge of 51.0 grains, gave an instrumental velocity at 78 feet of 2459 f. s. with a mean 10 pressure of 46,280 pounds per square inch.

While I have described only one composition, it will be understood by those familiar with the art that the proportions of nitroguanidine and nitrocellulose can be widely varied. While I have described simply the use of dinitrotoluene and specifically the 1, 2, 4-derivative, it will also be understood that I may use any deterrent material or mixture of deterrent materials having an appreciable solvent action on the nitrocellulose of the powder grain under the prevailing conditions. Deterrent materials which are suitable alone or in admixture are very numerous, but I will name only a few, such 25 as mononitronaphthalene, dinitrotoluene, trinitrotoluene, diethyldiphenylurea, etc.

I claim:

1. As a new propellant, a nitrocellulose powder containing nitroguanidine and having its surfaces impregnated with a deterrent material.
2. As a new propellant, a nitrocellulose powder containing nitroguanidine and having its surfaces impregnated with substantially pure 1, 2, 4-dinitrotoluene.
3. As a new propellant, a nitrocellulose powder containing nitroguanidine and having its surfaces impregnated with a nitrohydrocarbon.
4. As a new propellant, a nitrocellulose powder containing nitroguanidine and having its surfaces impregnated with a material having a solvent action on the nitrocellulose component of the powder grain.

5. As a new propellant, a nitrocellulose powder containing nitrocellulose and nitroguanidine and having its surface impregnated with a deterrent material, each 100 parts of nitrocellulose and nitroguanidine taken together comprising from about 30 to 80 parts of nitrocellulose, and from 70 to 20 parts of nitroguanidine.

6. As a new propellant, a nitrocellulose powder containing nitrocellulose and nitroguanidine and having its surface impregnated with dinitrotoluene, each 100 parts of nitrocellulose and nitroguanidine taken together comprising from about 30 to 80 parts of nitrocellulose, and from 70 to 20 parts of nitroguanidine.

7. As a new propellant, nitrocellulose powder grains containing about 60 parts of nitrocellulose, about 40 parts of nitroguanidine, and a deterrent material at the surface of said grains.

8. As a new propellant, nitrocellulose powder grains containing about 60 parts of nitrocellulose, about 40 parts of nitroguanidine, and dinitrotoluene at the surface of said grains.

9. As a new propellant, a nitrocellulose powder containing nitrocellulose of about 13% nitrogen content and nitroguanidine and having its surface impregnated with a deterrent material, each 100 parts of nitrocellulose and nitroguanidine taken together comprising from about 30 to 80 parts of nitrocellulose, and from 70 to 20 parts of nitroguanidine.

10. As a new propellant, nitrocellulose powder grains containing nitrocellulose of about 13% nitrogen content and nitroguanidine, the surfaces of said grains being impregnated with a deterrent material having a solvent action on the nitrocellulose component of said grains.

In testimony whereof I affix my signature.  
JOHN M. SKILLING.